

## UNITED STATES PATENT OFFICE

1,968,157

PROCESS OF PURIFYING VISCOSE  
SOLUTIONSWaldemar O. Mitscherling, Bridgeport, Conn.,  
assignor to The Pacific Lumber Company,  
Scotia, Calif., a corporation of MaineNo Drawing. Application August 13, 1927,  
Serial No. 212,836

18 Claims. (Cl. 260—100)

This invention relates to a method of purifying a solution used to produce artificial silk, artificial straw, artificial horsehair, films, and materials of like nature by extruding the solution through suitable spinnerets, dies or the like. It is particularly adapted for use in purifying viscose solutions (sodium cellulose xanthate solutions). In the practice of this invention the cellulose may be obtained from any source but it has been found that the process described herein is particularly advantageous where the cellulose is derived from the wood and bark of the redwood tree.

It has been found that if an amphoteric metal either in the metallic state or in combination, be added to the alkaline solution which is to be spun, that the amphoteric metal will react with the alkaline solution to give a metallic hydroxid and this further reacts to form an alkali metal salt of the amphoteric metal, and that this reacts further with certain of the organic constituents of the solution to give a gelatinous precipitate. For example, if the usual viscose solution is used and an amphoteric metal such as aluminum is added to this solution, a gelatinous precipitate will be formed which will carry down with it certain of the impurities and from which the clear solution may be separated by any desired means such as filtration or by subjecting it to centrifugal action. Simultaneously, with the formation by the metallic aluminum of the sodium aluminate, hydrogen gas is evolved.

If aluminum is employed the amount of aluminum which may be used varies according to the amount of impurities in the spinning solution and also according to the degree to which these impurities are desired to be eliminated. It has been found that an amount of aluminum between one-half of one per cent. and two per cent. by weight calculated on the cellulose content of the solution is satisfactory.

Although in the above example I have set forth the use of aluminum as the amphoteric metal which is to be employed, success can be similarly obtained by adding to the spinning solution other amphoteric metals either combined or uncombined and I have obtained satisfactory results by using zinc, zinc hydroxid, aluminum hydroxid, sodium zincate and sodium aluminate. The purification resulting is essentially the same no matter which of these materials is used. I prefer, however, to use zinc hydroxid or metallic aluminum.

By subjecting the spinning solution to the action of an amphoteric metal hydroxid, the remaining solution not only is purified but it has also been found is not subject to as rapid deterio-

ration as the unpurified solution. This is probably due to the precipitation of some of the usual decomposition products attendant upon xanthation.

The lustre of the rayon filaments made from this purified solution differs optically from rayon made from unpurified viscose solutions in that it does not reflect light from the surface so glaringly, but instead there is a translucent effect very similar to the appearance of silk from the silk worm cocoon.

The degree of purification thus effected may be controlled by the quantity of the amphoteric metal which is permitted to act on the solution. If the amphoteric metal be finely divided its action will be more rapid than if the metal be used in larger particles. In case finely powdered metal is employed it is of course necessary to guard suitably against too great a rise of temperature, say by adding the purifying agent slowly or by refrigeration.

The above described reaction when carried out produces a precipitate of a gelatinous or slimy nature containing the impurities and this precipitate forms a layer which can be removed, though with some difficulty, by means of a filter or by the action of a centrifuge or other similar device. A device which has proved particularly successful in separating these impurities from the spinning solution may consist of an ordinary cylindrical centrifugal separator containing a lining of amphoteric material such for example, as metallic aluminum or zinc. For example, a removable aluminum shell, preferably split so that it will tightly conform to the inside of the cylinder may advantageously be placed within a centrifuge of any usual type. In using a centrifugal separator in the practice of my process the spinning solution may be allowed to enter through the bottom of the cylinder and by the action of centrifugal force is whirled in contact with the amphoteric metal, which is used as a lining, and is withdrawn from the upper end of the cylinder. The centrifugal action of the process and the contact of the solution with the amphoteric metal gives rise to a chemical reaction between the materials in the spinning solution and the material of which the lining of the cylinder is formed in a manner similar to that which would take place if a finely powdered metal or compound of such metal were added to the spinning solution in a stationary container. The sludge formed on the shell by the action of the metal with the impurities in the spinning solution will gradually be carried toward the discharge end of the

60  
65  
70  
75  
80  
85  
90  
95  
100  
105  
110

centrifugal machine and is taken away through an outlet separate from that used to carry away the purified spinning solution.

Although I have set forth the preferred method 5 of practicing my invention, it is to be understood that changes may be made in the steps of the process and the materials employed without departing from the spirit of my invention or the scope of the subjoined claims.

10 I claim:

1. The method of purifying an alkaline cellulose solution which comprises effecting the reaction of an amphoteric metal hydroxid with a constituent of such solution adapted to combine with the 15 amphoteric metal to form a precipitate containing the impurities and removing said precipitate therefrom while the solution is still alkaline.

2. The method of purifying an alkaline cellulose solution which comprises effecting the reaction 20 of an amphoteric metal which will give an hydroxid with constituents of such solution adapted to combine with the amphoteric metal to form a precipitate containing the impurities and removing said precipitate therefrom while the solution is still alkaline.

3. The method of purifying an alkaline cellulose solution containing a compound of an alkali metal which comprises effecting the reaction of such alkali metal and an amphoteric metal 30 hydroxid and an organic constituent of the solution, and removing a product of such reaction therefrom while the solution is still alkaline, which product contains impurities formerly in the cellulose solution.

35 4. The method of purifying a cellulose solution containing a compound of an alkali metal which comprises effecting the reaction of such alkali metal compound and aluminum and an organic constituent of the solution and removing the 40 product of such reaction therefrom.

45 5. The method of purifying an alkaline cellulose solution containing a compound of sodium which comprises effecting the reaction of the sodium and an amphoteric metal hydroxid and an organic constituent present as an impurity in the 50 solution and removing the resulting precipitate containing said impurity therefrom while the solution is still alkaline.

6. The method of purifying a cellulose solution 55 containing a compound of sodium which comprises effecting the reaction of the sodium and metallic aluminum and organic constituents of the solution and removing a product of such reaction therefrom.

55 7. In a process of purifying alkaline cellulose solutions the steps of reacting upon a cellulose solution containing a compound of an alkali metal with an amphoteric metal hydroxid adapted to produce a gelatinous precipitate therewith said gelatinous precipitate being adapted to remove impurities from said solution, and separating said precipitate and said impurities from said solution while the solution is still alkaline.

65 8. In a process of purifying alkaline cellulose 70 solution the steps of reacting upon a cellulose

solution containing a compound of sodium with an amphoteric metal hydroxid adapted to produce a gelatinous precipitate therewith, said gelatinous precipitate being adapted to remove impurities from said solution, and separating said precipitate and said impurities from said solution while the solution is still alkaline.

80 9. The herein described process comprising reacting upon an alkaline viscose with an amphoteric metal hydroxid and separating the resulting precipitate containing impurities formerly present in said viscose therefrom while the solution is still alkaline.

85 10. The herein described process comprising reacting upon viscose with aluminum, and separating the resulting precipitate containing impurities formerly present in said viscose therefrom.

90 11. The method of purifying a viscose solution which comprises effecting the reaction of an amphoteric metal with constituents of such solution under the influence of centrifugal force to separate impurities present in said solution therefrom, and removing said impurities.

95 12. The method of purifying a viscose solution which comprises effecting the reaction of aluminum with constituents of such solution under the influence of centrifugal force to separate impurities present in said solution therefrom, and removing said impurities.

100 13. The method of purifying a viscose solution which comprises effecting the whirling of the solution in contact with a surface of an amphoteric metal.

110 14. The method of purifying a viscose solution which comprises effecting the whirling of the solution by a centrifugal action in contact with an aluminum surface.

115 15. The method of purifying an alkaline viscose solution which comprises effecting the reaction of an amphoteric metal with sodium and organic constituents present in the solution to produce a gelatinous precipitate and removing said precipitate therefrom while the solution is still alkaline.

120 16. The method of modifying the lustre of viscose rayon which comprises removing a portion of the lustre producing content of the alkaline viscose solution to be spun into rayon by the reaction of an amphoteric metal hydroxide upon a constituent of such solution and separating the resulting product while the solution is still alkaline.

125 17. In the manufacture of viscose products the step comprising treating alkaline viscose solution with metallic aluminum prior to spinning.

130 18. In the manufacture of viscose products the method of purifying alkaline viscose solution comprising treating said solution prior to spinning with a finely divided metallic metal 135 which is rapidly dissolved in alkali with liberation of hydrogen, dissolution of said metal destroying sulfur-compound impurities in the viscose solution.

140 WALDEMAR O. MITSCHERLING.